

April 18, 1944.

J. A. GUYER

2,346,750

## PROCESS FOR THE REACTIVATION OF CONTACT CATALYSTS

Filed April 14, 1941

2 Sheets-Sheet 1



INVENTOR  
JESSE A. GUYER

BY  
Hudson, Young, Shantz & Young  
ATTORNEY

April 18, 1944.

J. A. GUYER

2,346,750

PROCESS FOR THE REACTIVATION OF CONTACT CATALYSTS

Filed April 14, 1941

2 Sheets-Sheet 2



INVENTOR  
JESSE A. GUYER

BY  
Hudson, Young, Stanley & Genger  
ATTORNEY

## UNITED STATES PATENT OFFICE

2,346,750

PROCESS FOR THE REACTIVATION OF  
CONTACT CATALYSTSJesse A. Guyer, Bartlesville, Okla., assignor to  
Phillips Petroleum Company, a corporation of  
Delaware

Application April 14, 1941, Serial No. 388,535

4 Claims. (Cl. 196—52)

This invention relates to the catalytic treatment of hydrocarbons over contact catalyst masses to promote conversions commonly classified as cracking, reforming, dehydrogenation, cyclization, desulfurization, isomerization and the like. More particularly, this invention relates to an improved method and process for the reactivation of catalyst masses employed in said conversions and which are more or less progressively inactivated by the deposition of carbon and/or carbon-containing material on the catalyst particles.

In catalytic conversions of the type indicated, the nature of the reactants and the conditions of treatment are such that carbonaceous materials are formed and deposited on the catalyst mass, thereby impairing the catalyst activity. While the amount of carbonaceous material deposited may vary with the hydrocarbon stock undergoing conversion, the original activity of the catalyst, and the conditions, particularly the temperature of treatment, the ultimate result is a decrease in conversion to an economically unsatisfactory level. From the standpoint of product, quality and yield, it becomes necessary to reactivate the catalyst at suitable intervals corresponding to some predetermined standard or average value of economically satisfactory conversion.

In catalytic conversion processes wherein reactivation of the catalyst at relatively frequent intervals is necessary, it is common practice to incorporate into the plant design and equipment a sufficient number of catalyst-containing chambers so that a regular cycle of converting and reactivating operations is possible. Such a cycle ordinarily includes a treating period during which a unit volume of the catalyst is employed in the conversion and a reactivating period during which the said unit volume of catalyst is subjected in situ to controlled combustion conditions by the passage of an oxygen-containing gas at or above the ignition temperature of the carbonaceous deposits.

Reactivation of solid granular catalyst masses by combustion requires careful control of the rate of burning to prevent deterioration of the physical and catalytic properties thereof by excessive temperatures. Heat transfer within the catalyst mass is poor due to the non-conducting nature of the particles, and temperature control during combustion is usually attempted by the regulation of the oxygen content of the combustion atmosphere passed through the catalyst mass to thereby limit the exothermic heat generated. In this manner the combustion atmosphere may serve as

both the temperature control mechanism and the principal heat transfer medium.

The heat of combustion is primarily a measure of the amount of carbonaceous material burned, or in other terms, of the amount of oxygen admitted to the catalyst, and reactivation is ordinarily described as carried out in an atmosphere of relatively low oxygen content. The rate of combustion is thus to be limited and the exothermic heat to be controlled by the available oxygen in a unit volume of the combustion atmosphere. Also, during the period of reactivation it is often desirable to increase the oxygen concentration of the combustion atmosphere as the carbon content of the catalyst decreases to maintain a reasonably constant temperature and speed the reactivation operation.

However, the tremendous operating difficulties in such a procedure are centered in the regulation of the oxygen content of the combustion atmosphere. The oxygen content must be maintained at very low values which may be varied within known low limits during the reactivation period, and this degree of regulation has complicated the analytical and control procedures of the proposed reactivation processes in many cases to the point of inoperability. No ordinarily available gases have an oxygen content in the range required during the initial stages of reactivation. Thus, stack or spent combustion gases may have an average oxygen content of 5 to 10 or more volume per cent, while the combustion atmosphere required to reactivate a catalyst mass at temperatures below those causing catalyst deterioration should have an initial oxygen content in the range of 0.5 to 3 volume per cent.

Various methods have been proposed for producing and maintaining large volumes of gases of very greatly reduced oxygen content. It has been proposed, for example, to recycle the combustion atmosphere subsequent to passage through the catalyst undergoing reactivation as a source of substantially oxygen-free gas. Such recycle gas may then be blended with oxygen-containing gas in producing a combustion atmosphere of controlled oxygen content. This procedure is complicated by the fact that this recycle gas may have a substantial and fluctuating oxygen content at various intervals throughout the combustion period. Especially in the reactivation of catalysts disposed in multiple-tube reactors, the combustion may proceed unevenly due to unequal pressure drops in the various tubes so that the effluent gases from some tubes may contain substantially the original concentration of

oxygen while that from other tubes may be oxygen-free. Similarly, in catalyst vessels of relatively large cross-sectional area uneven combustion may result from uneven carbon deposition. This fact in turn requires a constant and accurate determination of the oxygen content of said recycle gas as long as it is being mixed with additional oxygen-containing gas ahead of the catalyst chamber. Such analysis is difficult to make, and the necessary continual re-proportioning of the gas streams being mixed introduces expensive and troublesome operating control. In addition to these difficulties, the recycle gas stream contains corrosive compounds such as hydrogen sulfide and sulfur dioxide and abrasive constituents such as dust which are destructive to compressors, blowers, control instruments and various other parts of the equipment of the system.

Thus, prior to recycling, the effluent combustion gas from the catalyst being reactivated is ordinarily chemically treated and/or scrubbed, dried, reheated and the like to remove components deleterious to the catalyst or to the reactivating equipment. A final disadvantage is the high carbon monoxide content of said recycled gases which, as hereinafter explained, is not desirable in the combustion atmosphere.

It has also been proposed to supply the required substantially oxygen-free gas in the form of steam. Such proposals are not feasible in many cases due to the high cost of providing the large amounts of steam required as well as to the frequent deleterious effects of high concentrations of steam on the catalyst. In the latter instance, control of the steam content as well as of the oxygen content of the combustion atmosphere leads to the multiplication of control problems and to the use of expensive cooling and reheating procedures to remove excess steam by condensation and to reheat the combustion atmosphere to ignition temperatures.

I have now discovered a method of conducting the reactivation of catalyst masses which from the standpoint of simplicity and economy of operation as well as the utilization of various novel features hereinafter described represents an important improvement in the art. My invention as exemplified in the control of the reactivation equipment and process has for its objects the elimination of the disadvantages formerly associated with catalyst reactivation by controlled combustion, and the employment of novel operating features and economics.

I have found that the removal of carbonaceous material from a catalyst mass may be expedited and more easily controlled by the use of a combustion atmosphere prepared by mixing an oxygen-containing gas with a substantially oxygen-free gas furnished from an external supply of substantially unvarying composition. I have further discovered a novel method of producing said substantially oxygen-free gas in any required volume and at a temperature level which makes its generation and use inexpensive and easily controlled. With this constant supply of substantially oxygen-free gas, I am able to control the reactivation process in all stages of combustion with ease and simplicity of equipment heretofore impossible. Other advantages of my process such as fuel economy and utilization of waste heat to generate steam and power for the process will be obvious from the following description.

I have noted that greatly improved results are obtained in reactivation by the use of a combustion atmosphere containing, in addition to a reg-

ulated oxygen content, maximum concentrations of carbon dioxide. The primary reactions involved when a gas containing oxygen is brought into contact with a carbon-coated bed of catalyst above ignition temperatures are the following, listed in molar equation form together with the heat of reaction, either evolved or absorbed:

- (1)  $C + O_2 \rightarrow CO_2 (+174,600 \text{ B. t. u.})$   
 (2)  $C + CO_2 \rightarrow 2CO (-70,200 \text{ B. t. u.})$

When water is formed or is present in the combustion atmosphere additional reactions are possible, as follows:

- (3)  $C + H_2O \rightarrow CO + H_2 (-70,900 \text{ B. t. u.})$   
 (4)  $C + 2H_2O \rightarrow CO_2 + 2H_2 (-71,600 \text{ B. t. u.})$   
 (5)  $CO + H_2O \rightarrow CO_2 + H_2 (-700 \text{ B. t. u.})$

Equation (1) represents the basic combustion reaction which is substantially instantaneous and is responsible for exothermic heat during reactivation. Equations (2) and (4) represent reactions which remove carbon from the catalyst and at the same time absorb heat. Equations (3) and (5) represent reactions which may be disregarded at the temperature levels of 600° to 1500° F. ordinarily employed in reactivation.

Reactions (2) and (4) are highly desirable in that they are endothermic and promote reactivation. To the extent that these reactions occur, reactivation is expedited, and the heat evolved by Reaction (1) is partly absorbed. Both effects are beneficial, and the latter even permits a slightly higher oxygen concentration in the combustion atmosphere. I have established the fact that Reaction (2) utilizing carbon dioxide is of far greater significance in this respect than Reaction (4) utilizing steam due to a greater reaction velocity at the above-mentioned temperature levels. Thus, carbon dioxide is superior to steam as a secondary reaction agent in the combustion atmosphere while the function of carbon monoxide as a product of the secondary reactions is to suppress the said desirable reactions. For these reasons I prefer to utilize a combustion atmosphere of closely controlled oxygen content prepared by mixing an oxygen-containing gas with a substantially oxygen-free gas also containing maximum quantities of carbon dioxide and minimum quantities of carbon monoxide. The concentration of steam in said combustion atmosphere may not exceed that present in ordinary flue or stack gases and may be limited to values consistent with operating economy and the susceptibility of the catalyst toward deterioration of steam.

In one specific embodiment, my process comprises the steps of (1) preparing a substantially oxygen-free gas by the combustion of fuel gas under moderate pressure in an atmosphere of oxygen-containing stack or spent combustion gases; (2) purging the catalyst space with substantially oxygen-free gas; (3) mixing the substantially oxygen-free gas with the stack gases or air to produce a mixture of limited oxygen concentration which is passed at suitable temperatures over the catalyst to be reactivated; (4) increasing the oxygen content of the combustion atmosphere as the reactivation proceeds to effectively maintain the rate of combustion; and (5) utilizing the sensible heat of the effluent gases from the catalyst chamber and of variable volumes of the excess gas produced by step (1) to generate steam and power for the operation of the process.

The various operations outlined may be illus-

trated by the flow diagrams of Figures 1 and 2 which show schematically two arrangements of equipment for the practice of my invention.

With reference to Figure 1, gas from stack 1, which may be part of a heater or furnace employed in the catalytic process is withdrawn through cooler 2 and line 3 to steam-driven compressor 4. The compressor delivers the gas through line 5 to pressure combustion chamber 6. In chamber 6 the stack gas is mixed with sufficient fuel gas from line 7 to produce combustion products substantially free of oxygen. The gas stream leaving chamber 6 is divided, passing through line 8 to line 10 which leads to the catalyst chambers 12, 13 and through the back-pressure regulator 9 to the waste heat boiler 11. The substantially oxygen-free gas passing through line 10 is thus available for uses requiring an inert atmosphere or for mixing with oxygen-containing gas. The latter may be stack gas from line 14 or in some cases air from line 15. The gases are introduced to the catalyst chambers through lines 16, 17 and 18.

The catalyst chambers are represented by two vessels although the number is not restricted and will vary according to the conversion being conducted. These vessels are fitted with inlet manifold lines 50 and 51 and outlet manifold lines 52 and 53 and vapor inlet line 54 and vapor outlet line 55 for the passage of hydrocarbons undergoing conversion, and also valves as shown for switching the flow of hydrocarbons and reactivating gases from one to the other of the vessels. The catalysts may be disposed in a single bed or in sections, on trays and the like, or in multiple tubes of relatively narrow cross section. The cycle of operations may be illustrated with two vessels although in actual operation with more vessels the time intervals of the various steps may overlap and be somewhat differently integrated.

Considering the catalyst in chamber 12 to be processing hydrocarbons, the catalyst in chamber 13 will be undergoing reactivation. The residual volatile hydrocarbons in chamber 13 are removed by purging with the substantially oxygen-free gas delivered through lines 10, 16, and 18, with the purged material exiting through lines 20, 21, and 22. The hydrocarbon vapors may be taken from line 22 to process equipment for recovery of the hydrocarbons.

After completion of the initial purging operation, reactivation is commenced by passing through chamber 13 a mixture of oxygen-containing stack gas from line 14 and substantially oxygen-free gas from line 10. The proportions of the mixture are regulated to produce the desired oxygen content. Assuming that a constant volume of gas is generated in combustion chamber 6, the requisite volume is delivered through line 10 by reduction of the flow through the back-pressure regulator 9. The effluent gas from chamber 13 passes through lines 20, 21 and 24 to the waste heat boiler 11. The gas stream leaving the boiler consists of the combined streams entering by lines 9 and 24, and passes through line 25 to vent 26.

The steam generated in the boiler 11 is withdrawn from the accumulator 27 through the pipe 28 and superheated in the heat exchanger 29 by heat exchange with the hot gases from pipe 10. The superheated steam is supplied to the prime mover 30 through the pipe 31. Steam from an external source may be admitted to the prime mover from the pipe 32 and used to augment the

supply from the waste heat boiler. The condensate from the prime mover 30 passes through trap 33 and line 34 to pump 35 which returns the condensate through line 36. Part of the water passing through line 36 is sent to boiler 11 as feed water through line 37 together with make-up water from line 38. Water is also injected into the combustion chamber 6 through line 39 for the purpose of cooling the combustion gas produced. Additional cooling of the gas passing through line 10 is obtained by water injection through line 40 and heat exchange in the heat exchanger 29.

The excess steam required over that produced in the waste heat boiler may be supplied from an external source as indicated, or may be produced wholly within the system by the supplementary combustion of fuel in boiler 11 by means of auxiliary burners not shown. These latter may also be useful in starting up the plant illustrated before waste heat from the gas streams is available.

As the reactivation proceeds, the oxygen concentration of the reactivating combustion atmosphere may be increased, and larger proportions of stack gas introduced through line 14. In fact, after the major portion of the carbonaceous residue on the catalyst has been oxidized, undiluted stack gas may be used, or still higher oxygen concentrations may be obtained by the introduction of air through line 15. In these latter stages, the temperature of the combustion atmosphere may be maintained at the desired levels by relatively small volumes of hot gases from line 10. When reactivation is complete, the catalyst chamber is again purged with substantially oxygen-free gas by closing lines 14 and 15 and passing only the stream from line 10 at the proper temperature. Thereafter the catalyst is ready to be placed in conversion service.

Figure 2 shows a modification of the apparatus in which the waste heat boiler is placed adjacent to or integral with the combustion chamber. In this fashion, the injection of water or steam to lower the temperature of the gas generated in said combustion chamber may be reduced or eliminated. The stack gas withdrawn from stack 1 passes through cooler 2 and line 3 to compressor 4. From the compressor the gas passes through line 5 to the combined combustion chamber and boiler unit 41 wherein combustion with fuel from line 7 is conducted to produce the substantially oxygen-free gas. Gaseous products of combustion pass through one tube bank of the boiler, which is divided by a partition 42, and the oxygen-free gas cooled by passage through the boiler tubes then passes to line 10.

Again considering the catalyst in chamber 13 to be undergoing reactivation, the catalyst bed is first purged of volatile hydrocarbons by means of substantially oxygen-free gas passing from the combustion chamber of unit 41 and through lines 10, 16, and 18 into chamber 13. The purged material exists through lines 20, 21, and 22.

The reactivating combustion is then commenced by passage of a mixture of substantially oxygen-free gas and oxygen-containing stack gas from lines 10 and 14. The temperature of the mixture is controlled by the volume of hot gas entering by line 10, and the oxygen content is regulated by the volume of stack gas from line 14. Any excess of gas in line 10 above that required for the mixture is vented through back-pressure regulator 9 to line 25 and vent 26. The effluent gas from chamber 13 passes through lines

20, 21, and 24 to the second tube bank of the unit 41, and thence through line 25 to vent 26.

The steam generated in the unit 41 is taken from accumulator 27 through lines 28 and 31 to the prime mover 30. Steam from an external source may be supplied through line 32. The condensate from the compressor engine is taken through trap 33, line 34 and pump 35, and returned to the unit 41 through heat exchanger 44 and line 36. Exchanger 44 serves as a feed water preheater and removes part of the heat added to the stack gas stream by the compression step. Boiler feed water from line 36 is passed to the unit 41 through line 37 together with make-up water from line 38. Water from line 36 may be injected through line 39 into the combustion chamber of the unit 41 if desired, although in most cases the necessary reduction in the temperature of the gas is accomplished in the boiler tubes.

Combustion of fuel in an atmosphere of stack gas is carried out in combustion chamber 6 and in unit 41 at moderate superatmospheric pressures of 15-50 pounds gauge or sufficient to maintain flow of the combustion atmosphere without further compression. The pressure of combustion may be only slightly below the discharge pressure of the compressor 4 which delivers the oxygen-containing stack gas to both the combustion chamber and the gas mixing lines ahead of the catalyst chambers. This condition conforms with equalization of pressure in the mixing operation and the use of the compressor to flow the combustion atmosphere through both the combustion chamber and the catalyst chambers. The system pressure from the compressor discharge to the outlet of the waste-heat boiler may be regulated within the indicated pressure range by suitable back-pressure regulators.

The combustion of fuel gas in an atmosphere of stack gas having an oxygen content lower than air and usually between 5 and 10 volume per cent produces a substantially oxygen-free gas of high carbon dioxide content at temperatures which are markedly lower than those resulting from the combustion of fuel gas in air. Thus with stack gases containing about 10 volume per cent of oxygen, the combustion temperature in chamber 6 is about 2400° F., whereas if air were used the temperature would be in the range of 3200-3500° F. This lowering of the temperature in chamber 6 is reflected in savings in the cost of construction and maintenance of chamber 6, because the higher temperatures cause more rapid deterioration of the shell, refractory linings, checker-work partitions and effluent gas lines.

The lower temperature of the gas generated in the pressure combustion chamber is also beneficial in the reduction of the degree of cooling which must be done to produce temperatures compatible with the various reactivation steps. For example, when it is desired to lower the temperature of the gas leaving chamber 6 to about 1400° F., the generation of said gas at 2400° F. instead of 3200° F. results in a reduction of about 50 per cent in the weight of steam required for the temperature reduction. When water is employed there is a corresponding reduction in the amount required. The temperature reduction at the outlet of chamber 6 may be done in two stages if desired. Thus water may be injected directly into the chamber through line 39 to reduce the gas temperature sufficiently to protect the line 8 and the portion of the gas passing through regulator 8 may be conducted to boiler

11 without further cooling. The gas stream passing through line 10 may be further cooled by additional water injected through line 40 prior to passage over the catalyst being reactivated.

5 In every case the degree of cooling of the gas in line 10 will be governed by the relative proportions of said gas used in the mixture with stack gas from line 14 and by the desired temperature of the said mixture at the inlet of the catalyst 10 chamber.

Instead of cooling the gas passed into the catalyst chambers 12, 13 and comprising the substantially oxygen-free gas issuing from chamber 6 or unit 41, by the injection of liquid water 15 through line 39, by the injection of liquid water through line 40, or by heat exchange in exchanger 29 with the steam issuing from accumulator 27, this gas may be cooled by the direct addition thereto of water in the form of steam. 20 The cooling steam may conveniently be made by the injection of steam as such before or after the blending with air or with stack gas.

The stack gas which serves as the combustion medium in chamber 6 and as the source of oxygen-containing gas in the combustion atmosphere is cooled to a temperature of about 100 to 300° F. ahead of the blower 4. The temperature rise, due to compression may be offset by a heat exchanger in the blower discharge and the heat

30 extracted may be utilized in any desired manner, for example, to preheat the feed water to the boiler as in the modification of Figure 2. The compressor output is regulated according to the gas requirements of the various phases of reactivation, with a constant volume ordinarily being supplied to the combustion chamber 6 or unit 41. The amount of fuel introduced is adjusted to the oxygen content of the stack gas, and the gas passing to pipe 10 is substantially 35 oxygen-free when the fuel added requires about 95 per cent or more of the oxygen present for combustion. In this type of operation a constant supply of substantially oxygen-free gas is available at all times without the necessity of any regulation to compensate for other variations throughout the system. Whatever excess of said substantially oxygen-free gas is produced is utilized in the production of steam.

The basic control of my process is reduced to 40 the proportioning of the gas streams which are mixed to prepare the combustion atmosphere. In its simplest aspects, the control comprises regulation of the valves or flow controllers in the lines 10, 14, and 15 to produce a gas mixture of 45 any desired oxygen concentration up to the maximum represented by the stack gases. Beyond this maximum, air may be used to produce any desired oxygen concentration up to the oxygen content of air. These ranges cover all ordinary 50 activation steps and indicate the flexibility and simplicity of operation of my process. Simple operating controls such as proportioning flow controllers actuated by the temperature of the effluent gas from the catalyst bed may be employed if desired.

The initial purge of the catalyst bed, prior to 55 reactivation is accomplished by discontinuing the flow of hydrocarbons, releasing the pressure on the vessel, and introducing substantially oxygen-free gas with or without added steam at a temperature usually approximating that employed during conversion. In some instances of treating very heavy material, subatmospheric pressures may be used to expedite removal of 60 hydrocarbons. While the purge gas may be

mixtures of substantially oxygen-free gas with steam, I often prefer to minimize the quantities of steam used on account of possible reactions occurring between the catalyst and steam which cause loss of catalytic activity.

After the catalyst bed is purged substantially free of volatile hydrocarbons, combustion is initiated by the introduction of gas containing low percentages of oxygen. The temperature of the catalyst may be raised or lowered by the purging operation, and the temperature of the oxygen-containing combustion atmosphere initially admitted is ordinarily regulated to minimum ignition temperatures in the range of 500° to 1000° F., depending on the type of catalyst, the nature of the catalytic conversion it has promoted and the maximum temperatures desired in reactivation. In general, the service or conversion temperature level will determine the reactivation temperature level for a catalyst. For example, catalysts used in reactions conducted at temperatures of 900° to 1300° F. may be reactivated at temperatures within that range or only slightly higher while catalysts used at temperatures of 600° to 900° F. are reactivated at substantially the same temperatures but not greatly exceeding 1200° F. In either case, the temperature at the beginning of the reactivation will be within the proper range, and with the control of the oxygen content of the combustion afforded by my process the maximum permissible temperatures are not exceeded.

In most cases, catalyst bed temperatures during reactivation will not exceed 1200° to 1400° F., and only in exceptional instances will temperatures above 1400° F. be tolerated without incurring catalyst deterioration. On the other hand, reactivation is often too slow and involves the handling of excessive volumes of combustion atmosphere when temperatures below about 500° to 700° F. are maintained.

Pressures in my process are moderate super-atmospheric pressures which may range from values at the blower discharge just sufficient to overcome the total pressure drop in the system to higher values of 150 pounds gauge or more maintained by pressure regulators on the effluent gas lines. In some cases, higher pressures are beneficial in shortening the final stages of reactivation.

The reactivating combustion may be divided into two phases according to the potential rate of combustion. The first or rapid phase includes the period required for removal of the surface coating of carbonaceous material from the catalyst granules. In this period the oxygen content of the combustion must be very low, generally of the order of 0.5 to about 3 volume per cent to prevent excessive temperatures at the combustion front or zone of intense oxidation. This zone is that portion of the catalyst bed in which previously mentioned Reaction (1) is occurring, involving the oxygen in the combustion atmosphere, and the temperature of this zone is governed by the concentration of oxygen. This zone and adjacent areas are also the sectors of the catalyst bed in which gasification of carbon by reaction with carbon dioxide and/or steam occurs. The gas passing through the combustion front is raised in temperature with the result that the entire bed is more or less gradually heated to a level which permits secondary reactions throughout the mass.

In my process the combustion front proceeds uniformly in the direction of reactivating gas

flow and eventually reaches the end of the catalyst bed. This terminates the first phase of reactivation. The second phase includes the combustion of carbonaceous material mostly beneath the surface of the catalyst granules, and higher oxygen concentrations in the combustion atmospheres are permissible and necessary to rapidly complete the reactivation. In this phase the weight of carbonaceous material removed is relatively small compared to the total weight originally present, and the rate of combustion is much slower. Oxygen concentration of the order of 2 to 10 per cent or more may be employed without producing excessive temperatures. In some cases, the final stages of reactivation may be carried out with air alone entering the catalyst bed.

The progress of the various phases of the reactivation may be measured by the temperatures at various points within the catalyst mass or by time measurements once the time periods of the successive operations have been established for a given operation. The time required for the actual combustion of carbonaceous material will depend on the weight of carbon on the catalyst, the type of catalyst and catalyst vessels and other factors involving the maximum desired temperatures during reactivation. In any case, adjustment of my process to any existing or desired set of conditions involves only proper control of the volume of the indicated gas streams being mixed at a single point in the system.

At the completion of the reactivating combustion which may be judged by the temperatures of the effluent combustion atmosphere or of the catalyst bed or by any conventional means, the flow of oxygen-containing gas is discontinued, and the catalyst is again purged with substantially oxygen-free gas to prepare said catalyst for further conversion service. This final purge may be of relatively brief duration, and the temperature of the purge gas may be regulated if desired to bring the catalyst bed to approximately conversion conditions. Thus, if the reactivation is completed at say 150° F. below or above conversion temperature, the purge gas may be utilized to raise or lower the catalyst temperature to the desired range. In this case, the catalyst may be placed on stream by introducing the hydrocarbon reactants and stopping the flow of purge gas.

Such expedients are of value in conversions such as catalytic cracking and the like wherein the complete cycle of operations with a unit of catalyst may not be longer than from one or less to about six hours.

The operation of the pressure combustion chamber as a source of substantially oxygen-free gas requires a minimum of regulating control. The oxygen content of the stack gas delivered to the chamber is essentially constant, and the quantity of fuel gas required to combine the oxygen present in a constant volume of said stack gas is thus fixed. The combustion temperature produced by stack gas containing about 10 volume per cent of oxygen is usually in the range of 2300 to 2500° F., and this range promotes complete oxidation of the fuel to carbon dioxide, whereas higher temperatures above 2800° F. may tend to promote the formation of carbon monoxide by both the combustion of the fuel and by the dissociation of carbon dioxide into carbon monoxide and oxygen. Thus the lower temperature of combustion obtained in my process produces a gas containing maximum concentrations of carbon dioxide substantially free of oxygen and carbon monoxide. In this respect, combustion is

more complete than when fuel gas is burned according to theoretical air requirements in air alone or in air diluted by steam.

Since the waste-heat boiler utilizes the excess of sensible heat of the hot effluent gas from the catalyst chambers, a large portion of the steam and power requirements is supplied by waste products of the process. The periods of maximum steam requirement correspond rather closely to the periods of maximum steam production since the largest volume of substantially oxygen-free gas is supplied to the catalyst during the initial combustion period when the temperature of the effluent gas is at a maximum. Conversely, the periods of minimum steam requirements correspond to the periods of minimum steam production. Excess steam requirements and steam for starting operations may be supplied as shown from an external source or may be generated in the waste-heat boiler by the auxiliary combustion of fuel gas and air therein or in the combustion chamber if desired.

The following specific examples will serve to illustrate applications of my process to the reactivation of catalysts used in specific conversions which differ greatly in respect to both conversion and reactivation conditions. Inasmuch as said examples are included to indicate the flexibility and operating advantages of my process, no limitation is implied thereby.

#### Example I

A catalytic gas-oil cracking operation was conducted with a silica-alumina type catalyst under conditions such that the conversion-reactivation cycle was six hours. Of this cycle, the conversion period was two hours during which carbon deposition amounted to approximately 2 per cent by weight of the gas-oil charge. Three catalyst chambers were employed in the operation, and the reactivation equipment was substantially the same as shown in Figure 2 except that gas mixing manifolds were provided for the individual chambers.

After the catalyst in the first chamber completed 2 hours of conversion, the flow of hydrocarbon reactants was switched to the second chamber. The pressure on said first chamber was released and substantially oxygen-free gas delivered from the pressure combustion chamber at about 2400° F. and cooled to about 950° F. was introduced for the initial purge gas. The flow of purge gas and hydrocarbon vapors was directed to a scrubber wherein the hydrocarbons were separated.

The initial purge was complete after 30 minutes, and with the catalyst at approximately 950° F., the combustion was initiated by introducing a mixture of stack gas with sufficient substantially oxygen-free gas to produce an oxygen content of about 2 volume per cent. This initial mixture was 20 per cent of stack gas and 80 per cent substantially oxygen-free gas, and was prepared by mixing 80% oxygen-free gas from the pressure combustion chamber with 20% cooled stack gas containing about 10% oxygen to produce a mixture temperature of about 900° F.

After a period of 1.5 hours, the initial combustion phase was complete with the maximum temperature not substantially exceeding 1100°-1200° F. and the temperatures of the catalyst mass showed that the combustion front had traversed the bed. At this point, the oxygen content of the combustion atmosphere was raised to about

5 per cent by mixing equal volumes of cooled stack gas and substantially oxygen-free gas from the combustion chamber. This second phase of combustion was continued for 1.5 hours or until reactivation was completed. The catalyst chamber was then purged with substantially oxygen-free gas at a temperature of 950° F. for about 30 minutes to remove the oxygen, and the catalyst was again put on stream.

During the above-described reactivation, the said second chamber was removed from conversion service at the end of 2 hours for reactivation, with the third chamber being put on stream. The sequence of reactivation operations thus over-lapped with the initial purge and initial combustion period of said second chamber occurring simultaneously with the final combustion period and final purge of said first chamber. By this scheme of operation the volume requirements for each of the gas streams used in the sequence of reactivating steps remained essentially constant.

#### Example II

A bauxite catalyst used in the desulfurization of cracked gasoline vapors at 750° F. was reactivated after 12 hours on stream. With this extended period of service, dual catalyst chambers of relatively large cross-section were provided and the reactivation was completed in about 9 hours. The catalyst to be reactivated was purged free of gasoline vapors by means of a mixture of substantially oxygen-free gas prepared as in the foregoing and steam at a temperature of about 700° F. The purged catalyst was then reactivated for a period of 7 hours with a combustion atmosphere composed of stack gas and said substantially oxygen-free gas and steam entering the chamber at about 850° F. During reactivation, the oxygen content of the combustion atmosphere was gradually increased from 2.5 per cent to 10 per cent, with the first increase coming after 4 hours. Maximum temperatures within the catalyst bed did not substantially exceed 1400° F. at any period and during the last 2 hours of the 9 hour period the inlet temperature of the combustion atmosphere was raised to 900° F. The reactivation was completed in 9 hours, and the chamber was purged again with substantially oxygen-free gas and steam at a temperature of about 750° F. to eliminate oxygen.

My invention is not limited to the reactivation of any particular type of catalyst nor to any specific conversion in which catalysts are deactivated by the deposition of carbonaceous deposits. In general, the catalysts to be reactivated according to the terms of the foregoing disclosure are those which are restored to a suitable activity under the specified controlled conditions but which are susceptible to deterioration if the said specified conditions are exceeded during reactivation treatment. Examples of such materials are the various contact catalysts classified as clay-type and mineral ore materials and natural or synthetic metal oxides including the difficultly reducible oxides alone or in mixtures with each other and/or promoted with other metals or metal salts. Specific examples are bauxite and bauxite impregnated with chromium, zirconium, and other oxides used in cracking, dehydrogenation, aromatization and desulfurization conversions and composite catalysts prepared from silicon and aluminum oxides and activated silicates.

The term "stack gas" and "spent combustion gas" as employed in the foregoing disclosure are intended to designate the gases produced by the combustion of fuels with moderate amounts of excess air according to conventional procedures known to the art. Such gases ordinarily comprise carbon dioxide, nitrogen, oxygen and water vapor with the relative amounts of these and other minor components varying according to the type of fuel and the efficiency of the combustion operation.

The term "moisture" as used in certain of the appended claims includes water in the form of either liquid water or steam.

Having thus described my invention, I claim:

1. A method of regenerating a catalyst of reduced activity by removing combustible deposits from the catalyst which comprises burning fuel in an atmosphere of an oxygen-containing stack gas, the latter containing a substantial amount but not over 10 volume per cent of oxygen and prepared by the combustion of fuel with a limited amount of excess air, the proportions of said fuel and said stack gas being so adjusted to produce a substantially oxygen-free and carbon monoxide-free gas, mixing the resultant substantially oxygen-free and carbon monoxide-free gas with an oxygen-containing gas to form a regenerating gaseous mixture having an oxygen content of less than 10% by volume, and introducing said mixture into contact with the catalyst to regenerate the catalyst by removal of combustible deposits from the catalyst.

2. A method of regenerating a catalyst of reduced activity by removing combustible deposits from the catalyst which comprises burning fuel in an atmosphere of stack gas, the latter containing a substantial amount but not over 10 volume per cent of oxygen and prepared by the combustion of fuel with a limited amount of excess air, the proportion of said fuel and said stack gas being so adjusted to produce substantially oxygen-free and carbon monoxide-free gas, mixing the resultant substantially oxygen-free and carbon monoxide-free gas with controlled amounts of said stack gas to form a regenerating

gaseous mixture having a controlled oxygen content of less than 10% by volume, introducing the said mixture into contact with the catalyst to regenerate the catalyst by removal of combustible deposits from the catalyst, and adding moisture to the regenerating gaseous mixture to limit the temperature of the regeneration below a predetermined maximum.

3. A method of making a gas suitable for regenerating a catalyst of reduced activity by removing combustible deposits from the catalyst which comprises burning fuel in an atmosphere of stack gas, the latter containing a substantial amount but not over 10 volume per cent of oxygen and prepared by the combustion of fuel with a limited amount of excess air, to produce a substantially oxygen free and carbon monoxide-free gas, and mixing the resultant substantially oxygen-free and carbon monoxide-free gas with air to form a mixture of combustion products and oxygen having an oxygen content of less than 10% by volume.

4. In a process for the reactivation of solid contact catalysts employed in the conversion of hydrocarbons, the activity of which has been substantially reduced by the deposition of oxidizable carbonaceous material thereon, which comprises passing a portion of a gas into contact with the catalyst to purge the catalyst of hydrocarbon vapors, mixing another portion of said gas with oxygen-containing combustion products to produce a mixture of suitable reduced oxygen content, and passing said mixture into contact with said catalyst to effect removal of the carbonaceous material by combustion and gasification of said material, the improvement which comprises generating said gas by burning fuel gas in an atmosphere of combustion products having a substantial content but not over 10 volume per cent of oxygen, the proportions of said fuel and said combustion products being so adjusted to produce a gas containing carbon dioxide and substantially free of oxygen and carbon monoxide.

JESSE A. GUYER.

CERTIFICATE OF CORRECTION.

Patent No. 2,346,750.

April 18, 1944.

JESSE A. GUYER.

It is hereby certified that error appears in the printed specification of the above numbered patent requiring correction as follows: Page 3, second column, line 52, for "ins" read --line--; line 64, for "exists" read --exists--; page 5, second column, line 7, for "atmospheres" read --atmosphere--; line 47, for "thise" read --this--; page 7, first column, line 1, for "term" read --terms--; and that the said Letters Patent should be read with this correction therein that the same may conform to the record of the case in the Patent Office.

Signed and sealed this 29th day of August, A.D. 1944.

Leslie Frazer  
Acting Commissioner of Patents.

(Seal)

CERTIFICATE OF CORRECTION.

Patent No. 2,346,750.

April 18, 1944.

JESSE A. GUYER.

It is hereby certified that error appears in the printed specification of the above numbered patent requiring correction as follows: Page 3, second column, line 52, for "ine" read --line--; line 64, for "exists" read --exists--; page 5, second column, line 7, for "atmospheres" read --atmosphere--; line 47, for "thise" read --this--; page 7, first column, line 1, for "term" read --terms--; and that the said Letters Patent should be read with this correction therein that the same may conform to the record of the case in the Patent Office.

Signed and sealed this 29th day of August, A.D. 1944.

(Seal)

Leslie Frazer  
Acting Commissioner of Patents.